

T. W. CASE,  
PHOTO-ELECTRIC CELL,  
APPLICATION FILED AUG. 27, 1920.

1,376,605.

Patented May 3, 1921.

Fig 1.



Fig 2.



T. W. Case, INVENTOR  
BY  
Duncan Thompson, ATTORNEY

# UNITED STATES PATENT OFFICE.

THEODORE W. CASE, OF SCIPIO, NEW YORK.

## PHOTO-ELECTRIC CELL.

1,376,605.

Specification of Letters Patent.

Patented May 3, 1921.

Application filed August 27, 1920. Serial No. 406,463.

*To all whom it may concern:*

Be it known that I, THEODORE W. CASE, of Scipio, in the county of Cayuga in the State of New York, have invented new and useful Improvements in Photo-Electric Cells, of which the following, taken in connection with the accompanying drawings, is a full, clear, and exact description.

This invention relates to certain improvements in photo-electric cells.

The object of the invention is to produce a highly efficient cell of the character described, and which shall be of simple construction, unusually constant and uniform in reaction, and relatively permanent in its activity.

Other objects and advantages relate to the details of construction of the cell, all of which will more fully appear from the following description, taken in connection with the accompanying drawings, in which:—

Figure 1 is a diagrammatic view illustrating a method of carrying out one step of the process of producing the cell.

Fig. 2 is a diagrammatic view illustrating a manner of use of the cell of this invention.

The completed cell of this invention consists of a vacuum tube inclosing a plurality of electrodes, one of which is provided with a coating of barium deposited thereon in a manner to be hereinafter described.

The invention, however, contemplates and permits of the introduction of a quantity of an inert gas, such as argon or helium, into the vacuum tube containing the electrode.

Under such circumstances, it may be suggested that the photo-electrons emitted by the action of light ionize the inert gas by impact resulting in maximum conductivity.

It is believed at present that the constant and uniform re-action of the cell, its relative permanency of activity and great intensity are largely the result of the peculiar structural form of one of the electrodes of the cell due to the peculiar and novel method of manufacture.

The physical structure of the coating of metal deposited upon one of the electrodes is not at present known with absolute certainty, and the theory of the action that results in the unexpected sensitivity of the element so produced is more or less a matter for intelligent speculation, and the applicant hesitates to state positively any definite

theory, and desires to confine himself to the demonstrated fact that the element so produced is highly sensitive and relatively permanent in its activity, but with this reservation, it may be suggested as indicative of applicant's present theory, that the metal deposited in the form of a coating upon one of the electrodes is in a peculiar structural condition resultant from the fact of its deposit in the manner to be described under constant bombardment by cathode rays or electrons.

The process of manufacture described and claimed in my co-pending application, Serial No. 406,462, comprises primarily the coating of an electrode capable of being heated, such as a filament with barium oxid. This coating may be produced upon the filament in any suitable way, as by dipping the same in barium nitrate at a suitable temperature to cause the same to flow upon the filament, and, by increase in temperature, change the nitrate to an oxid.

The coated filament is then placed in an ordinary glass tube or bulb opposite a metallic electrode, as, for instance, a nickel plate. The bulb is then evacuated and the whole is baked at such a temperature as may be suitable for eliminating practically all traces of gases. Then the filament and metallic electrode are preferably connected in a circuit with a source of sufficiently high potential so as to heat the metallic electrode red hot, thus driving off from the metallic electrode any remaining traces of gases and oxygen.

The electrode temperature is then reduced by regulating the potential to that found by experiment most suitable under the circumstances for the particular operating conditions without heating the electrode to a red heat. A suitable circuit is provided containing a source of potential for heating the filament to such a temperature as will result in throwing off the said filament coating in the form of relatively small particles.

By connecting the filament and metallic electrode in a circuit containing a suitable source of potential, the thrown-off material of the coating applied to the filament is, to a very large extent, caused to be deposited upon the metallic electrode. In other words, the high potential existing between the electrodes acts as a directive agency and causes the thrown-off material to deposit upon the

plate in a thin layer, where it is continuously bombarded by the cathode rays, or electrons, emanating from the filament and directed by the potential of the metallic electrode.

It is found that when a filament, as described, is coated with barium oxid, that the oxid is lost when the material is finally deposited on the metallic electrode, and that the deposit upon the metallic electrode is a coating of substantially pure barium.

Although a high potential direct current is suitable for the purpose described, the applicant in his work has usually incorporated a transformer in the circuit whereby the potential of the alternating current available was stepped up to an extent suitable for most effectively acting as a directive agency of the material thrown off from the filament, as well as producing a bombardment by cathode rays of the material deposited on the plate. During this step of the operation, the tube or bulb is connected to a suitable vacuum pump for maintaining a substantially complete vacuum within the bulb.

This condition may be maintained for stated intervals, as, for instance, five minute periods, and after each such period the photo-electric qualities of the cell may be tested in comparison with a constant source of light, and when the maximum re-action is obtained, the vacuum pump may be shut off and the tube containing the filament and metallic electrode sealed.

During the process of manufacture when using a direct current the potential in the circuit is so arranged as to maintain a positive potential upon the metallic electrode and a negative potential upon the filament.

In Fig. 1 I have diagrammatically illustrated a hook-up suitable for carrying out the depositing step of this process in which the filament —1— is connected in an independent heating circuit —2— with a source of potential —3— and in which the circuit between the filament —1— and metallic electrode —2— includes the secondary —4— of a transformer, the primary —8— of which is connected in circuit with a suitable source of alternating current. The secondary of the transformer embodies a considerably larger number of coils than the primary to produce desired voltage. When the process of producing the cell is completed, as described, the filament is thereafter used only

as an unheated electrode, and any other form of electrode may be substituted.

In Fig. 2 I have illustrated the cell in a hook-up suitable for measuring light intensity in which two electrodes are connected in circuit with a source of potential —7— and a galvanometer —5—. Variations in the light rays to which the cell (which includes the electrodes —1— and —2— and the vacuum tube or bulb —6—) is exposed, will be accurately indicated in a known standard of measurement by the galvanometer —5—.

The process above described permits of practically perfect control in the manufacture of cells of uniform action. Further, the method offers a substantially perfect control in obtaining the desired spectral sensitivity of the cell by combining the proper substances on the filament to be deposited on the metallic electrode, and by permitting control of the deposition by proper potential between the electrodes and proper temperature.

What I claim is

1. A photo-electric cell including an electrode having a coating of barium.
2. A photo-electric cell including an electrode comprising barium.
3. A photo-electric cell including an electrode having a thin coating comprising barium.
4. A photo-electric cell including an electrode having a coating of barium deposited under bombardment by cathode rays.
5. A photo-electric cell including an electrode comprising barium deposited under bombardment by cathode rays.
6. A photo-electric cell including an electrode having a thin coating comprising barium deposited under bombardment by cathode rays.
7. A photo-electric cell comprising a plurality of electrodes, one of which is of filamentary form.
8. A photo-electric cell comprising a filamentary electrode and an electrode comprising light sensitive material thrown off from the filament and deposited on the other electrode under bombardment by cathode rays.

In witness whereof I have hereunto set my hand.

THEODORE W. CASE

Witnesses:

EARL L. SPONABLE,  
JOHN TABER.